

## UNITED STATES PATENT OFFICE

2,600,058

## LUBRICANT CONTAINING SOAP OF PHOSPHATED HYDROXY FATTY ACID OR GLYCERIDE

Edwin C. Knowles, Glenham, Oney P. Puryear, Fishkill, and George W. Eckert, Glenham, N. Y., assignors to The Texas Company, New York, N. Y., a corporation of Delaware

No Drawing. Application March 9, 1949,  
Serial No. 80,574

11 Claims. (Cl. 252—32.5)

1

This invention relates to a lubricating composition and particularly a lubricating grease prepared from a soap of a phosphated hydroxy fatty acid or glyceride.

One of the principal objects of the present invention is to provide a lubricating composition containing as an additive to improve the lubricating characteristics thereof a metal soap of a phosphated soap-forming hydroxy fatty acid or glyceride thereof, such as phosphated castor oil or phosphated hydrogenated castor oil.

Another object of the invention is to provide a lubricating grease comprising an oleaginous liquid lubricating base containing a sufficient proportion of a soap of a phosphated hydroxy fatty acid or glyceride of this character to thicken the lubricating base to a gel-like consistency.

Other objects and advantages of the invention will be apparent from the following description and the accompanying claims.

In accordance with the present invention, a novel type of metal soap of a phosphated hydroxy fatty acid or glyceride is employed as an additive to impart enhanced lubricating characteristics or to thicken the mineral lubricating oil or other oleaginous liquid lubricating base to a gel-like consistency to form a lubricating grease. In the preparation of this additive or soap, the various soap-forming hydroxy fatty acid glycerides and their corresponding hydroxy fatty acids are first modified by phosphorylation to substitute a pentavalent phosphate group for the hydroxy group of the glyceride or acid with the splitting off of water. This produces a complex compound containing both the carboxylic acid radical (as a glyceride where the starting material is a glyceride) and the phosphate acid radicals. The resulting compound is then reacted with a sufficient proportion of a basic metallic compound, such as an oxide or hydroxide, for neutralization of the phosphate radical and for saponification of the glyceride or fatty acid radical.

Examples of suitable hydroxy fatty acids which are phosphated to produce the phosphated compounds of the present invention are the hydroxy-stearic acids, such as 12-hydroxystearic acid, hydroxymyristic acid, hydroxypalmitic acid, hydroxybehenic acid and ricinoleic acid. Likewise, the corresponding glycerides of these hydroxy fatty acids can be employed, it being understood that glycerine is liberated in the neutralizing step with the production of the same type of metal soap of the complex phosphated hydroxy fatty acid. As representative of a readily available and economical supply of the raw soap-

forming fatty material, phosphated castor oil and phosphated hydrogenated castor oil are specifically mentioned. In the following description, phosphated castor oil will be specifically discussed by way of preferred example, but it is to be understood that the invention applies in the same manner to the phosphated hydrogenated castor oil and to the phosphated hydroxy fatty acids enumerated above.

10 Castor oil contains the glyceride of ricinoleic acid, an unsaturated hydroxy C<sub>18</sub> acid, having the formula



15 Phosphated castor oil has the phosphate group linked to the glyceride of ricinoleic acid by replacing the hydroxy group in the 12-position, as follows:



A phosphated castor oil product available commercially gives the following tests:

30 Neutralization number ----- 135 to 160  
Saponification number ----- 290 to 310  
Iodine number ----- 75 to 80  
Phosphorus (total), per cent ----- 3.5 to 4.6

35 This commercial product contains about 45 to 50% by weight of phosphated castor oil and 55 to 50% castor oil.

40 In preparing the soap, sufficient basic material is employed to react with and neutralize both the carboxylic and phosphoric acid groups, thus giving



in the case of sodium soap. When castor oil is hydrogenated, the glyceride of the unsaturated ricinoleic acid is converted to the glyceride of the saturated 12-hydroxystearic acid, and the latter gives the corresponding phosphated 12-hydroxystearic acid glyceride which is then neutralized in a similar manner.

50 Whenever the expressions "phosphated soap-forming material," "phosphated soap-forming hydroxy fatty acid," "phosphated soap-forming

hydroxy fatty acid glyceride," "phosphated castor oil," "phosphated hydrogenated castor oil" and similar expressions are employed in the following description and claims, it is to be understood that each designates the type of compound described above wherein a pentavalent ortho-phosphate group has been substituted for a hydroxy group attached to the carbon chain remote from the carboxyl group of the hydroxy fatty acid or glyceride thereof, with the splitting off of water. The resulting phosphated compound thus contains the unmodified COOH group of the hydroxy fatty acid (or the corresponding glyceride thereof) as well as unneutralized OH radicals of the ortho-phosphate group, with both the COOH group and the OH radicals of the orthophosphate group of the compound being available for neutralization in the formation of the metal soap.

Alkali, alkaline earth, and polyvalent metal soaps of the phosphated hydroxy acids can be employed in accordance with the present invention in relatively small proportions of the order of 0.1-5.0% or greater in a mineral lubricating oil as an additive to impart enhanced lubricating properties. Low concentrations of these soaps in lubricating oil to provide a liquid lubricant impart added body, greater load carrying capacity (extreme pressure properties), and better corrosion and rust resistance as compared with the base oil. As specific examples, an improved textile lubricant is produced by the addition of about 0.5-2.0% of the sodium soap of phosphated castor oil to a mineral lubricating oil having a SUS. viscosity at 100° F. of about 50-120 to give a heavier bodied oil; and, for protective coatings, the addition of about 1.5-5.0% of the calcium or other alkaline earth or heavy metal soap of the phosphated castor oil to a similar mineral lubricating oil can be employed to give products having a definite yield point or even a gel-like structure.

Moreover, the metal soaps, particularly those of such elements as sodium, lithium, magnesium, zinc and aluminum and the mixed base soaps, such as sodium-calcium and sodium-lead, have been found to produce lubricating greases having advantageous, and in certain respects, unusual properties when added in sufficient proportion to thicken the mineral lubricating oil or other oleaginous liquid lubricating base to a gel-like consistency. Ordinarily, a proportion of soap in excess of about 5% up to about 40-45% by weight on the weight of the grease composition is employed to produce greases meeting the specifications of the different grades. Any of the various mineral lubricating oils customarily employed for grease making, as well as the various types of synthetic liquid oleaginous lubricating bases having comparable viscosities can be employed as part or all of the lubricating base with these particular soaps. Among the types of synthetic oleaginous liquid lubricating bases which are suitable may be mentioned the oil-soluble high boiling high molecular weight aliphatic ethers, aromatic esters, aliphatic mono- and dicarboxylic acid esters, phosphorus acid esters and halogenated aromatic compounds which possess lubricating properties and also have small change in viscosity for a given change in temperature. Of the various synthetic oleaginous compounds specified, those falling within the category of aliphatic dicarboxylic acid esters and particularly the branched chain aliphatic esters, such as di-2-ethylhexyl sebacate, are preferred. In the following description and claims, the expression "oleaginous

liquid lubricating base" is employed to designate both the mineral lubricating oils and the synthetic lubricating bases specified.

In the preparation of a grease in accordance with the present invention, the particular phosphated hydroxy fatty acid or glyceride is heated with a metal oxide or hydroxide in the presence of water and a portion or all of the mineral lubricating oil or other liquid oleaginous vehicle at a temperature of about 175-240° F. for a period of about 1-2 hours, utilizing sufficient of the metallic base to effect complete neutralization of the acid groups of both the phosphate radical and the carboxylic acid radical. Following this saponification period the product is then dehydrated by heating at a higher temperature up to about 300-330° F. for a further period of about 1/2-3 hours. Any further oil addition is made to the saponified product during dehydration, or following dehydration and as it gradually cools, with continual stirring to obtain the desired consistency; and additional ingredients or additives, such as antioxidants, anti-corrosives, extreme pressure agents, dyes and the like, can be incorporated. The product is ordinarily drawn after cooling to a temperature of about 200-100° F. to provide the ultimate gel-like grease.

Also, in accordance with the present invention, the properties of the resulting phosphated hydroxy acid soap grease can be desirably modified by utilizing a mixture of the phosphated hydroxy fatty acid or glyceride with a conventional soap-forming fatty acid or glyceride for the saponification step. Any of the ordinary saturated and unsaturated soap-forming fatty acids and fats or of the hydroxy fatty acids or hydroxy fats, including the hydrogenated fats and fatty acids, such as hydrogenated fish oil acids, can be employed for this purpose. A mixture consisting essentially of substantial portions each of the phosphated hydroxy fatty acid or glyceride and an unmodified hydroxy fatty acid or glyceride, as well as the foregoing mixture in major proportion together with a minor but modifying proportion of a conventional soap-forming fatty acid, have been found particularly advantageous in accordance with the present invention. In addition to saponifying a mixture of the phosphated hydroxy acid and other carboxylic acid with the desired metal base or mixture of metal bases, satisfactory greases can also be produced by separately performing the two or more types of soap specified and then mixing them with the addition of further oleaginous liquid lubricating base to produce a grease of the required consistency.

The following examples are set forth as representative and illustrative of the present invention:

#### EXAMPLE I

A sodium base grease of phosphated castor oil was prepared as follows: 200 grams of water, 375 grams of a naphthene base lubricating oil having an SUS. viscosity at 100° F. of 307, and 370 grams of the above mentioned commercial phosphated castor oil containing 3.7% by weight of combined phosphorus and having a neutralization number of 156, a saponification number of 295 and an iodine number of 79, were charged to a grease kettle, and heating and stirring were initiated. When a temperature of the kettle contents of 200° F. had been reached, 157 grams of a 50% aqueous solution of sodium hydroxide was added dropwise over a period of 1/2 hour, and an additional 100 grams of rinse water was added in a further period of 5 minutes. The saponification reaction

was continued at 200-206° F. for a further period of 1 hour. The temperature was then gradually raised to 300° F. over a period of 3/4 hour, and a further quantity of 1900 grams of the said naphthalene base lubricating oil was introduced slowly. Then heating and stirring at about 300-309° F. for dehydration with continued oil addition was carried out over a period of about 4 hours, when a control sample taken for penetration showed an ASTM unworked penetration of 123 at 77° F. and a worked penetration of 210 at 80° F. The heat was then cut and the temperature dropped slowly with continued stirring to about 210° F. over a period of 1 1/4 hours. A solution of 13.5 grams of diphenylamine in 50 grams of the naphthalene base lubricating oil, together with 500 grams additional of the lubricating oil were then slowly added at this temperature over a period of 3/4 hour. The resulting product was then drawn to obtain an excellent yield of a transparent light yellow stiff buttery grease.

A series of other metal soap greases of the commercial phosphated castor oil, including a lithium base grease, a magnesium base grease, a zinc base grease, an aluminum base grease, a 3:1 sodium-calcium mixed base grease and a 3:1 sodium-lead mixed base grease were also prepared in a similar manner and utilizing the same naphthalene base lubricating oil. Typical tests and the characteristic appearance of the above described sodium base and the other metal base greases so obtained are set forth in the following Table I:

Table I

| Metal          | Soap, Percent Calculated | Drop Pt., °F. | ASTM Penetration, Unworked | 77° F. Worked | Appearance                                                            |
|----------------|--------------------------|---------------|----------------------------|---------------|-----------------------------------------------------------------------|
| sodium         | 13.5                     | 485           | 144                        | 293           | transparent light yellow, stiff, buttery, clear amber, light feather. |
| lithium        | 12.6                     | 500+          | 138                        | 269           | transparent amber, stringy.                                           |
| magnesium      | 20                       | 340           | 275                        | 344           | opaque ivory, soft, buttery.                                          |
| zinc           | 20                       | 233           | 201                        | 274           | amber, transparent gel.                                               |
| aluminum       | 23.8                     | 224           | 191                        | 249           | transparent pale yellow, hard, buttery.                               |
| sodium-calcium | 10                       | 407           | 128                        | 273           |                                                                       |
| sodium-lead    | 15                       | 268           | 157                        | 286           |                                                                       |

In addition to the foregoing tests for dropping point and penetration, other tests were obtained on this series of greases as set forth in appended Table II:

Table II

|                                                       | Na | Li  | Mg | Zn | Na:Cu | Na:Pb |
|-------------------------------------------------------|----|-----|----|----|-------|-------|
| Dynamic Shear Test, Miniature Penetration:            |    |     |    |    |       |       |
| Original                                              | 41 | 45  |    |    | 40    | 83    |
| Final                                                 | 34 | 113 |    |    | 35    | 36    |
| Lubrication-Grease Breakdown Machine—R. T. to 300° F. |    |     |    |    |       |       |
| Low-Temperature Torque, sec./rev.:                    | A  | E   | E  | E  | E     | E     |
| Minus 20° F.                                          | 18 |     |    |    | 11.8  | 19.6  |
| Minus 30° F.                                          | 67 | 87  |    |    | 62.5  | 94.3  |
| Lubrication-Torque Breakdown Machine:                 |    |     |    |    |       |       |
| Timken Bearing 80° F.                                 | F  | E   | E  | E  | E     | E     |
| Timken Bearing 80-250° F.                             | G  | E   | E  | P  | E     | E     |
| Federal Bearing 80° F.                                | G  | E   | G  | G  | E     | E     |
| Federal Bearing 80-250° F.                            | F  | G   | E  | P  | G     | G     |

70

<sup>1</sup> Letters denote: E—excellent; G—good; A—adequate; F—fair; P—poor.

The dynamic shear resistance test of the foregoing table is a measure of the resistance of the

grease to texture change when worked under high shearing stress, the test being carried out as described in U. S. Patent No. 2,450,219, Ashburn and Puryear, in column 5, lines 6-19. A small change in miniature penetration of the sample after test in comparison with the original is indicative of excellent texture stability under high shearing stress. The miniature penetration test is described in Ind. Eng. Chem., Analytical Edition, vol. II, page 108, February 15, 1939.

The grease breakdown machine test is used to determine the lubricating properties of ball bearing greases at various temperatures. The machine employed consists essentially of a standard motor-driven rotating ball bearing (20 mm. bore x 47 mm. diameter x 14 mm. width) mounted vertically and enclosed in an oil jacket containing an electric immersion coil with adjustable rheostat for temperature control. The upper face of the bearing is not covered, so that observations of performance during operation can be made. The bearing is charged with 5 grams of the grease initially. With the system at atmospheric temperature, rotation of the packed test bearing is started at 3450 R. P. M. and allowed to proceed for 3 minutes, during which time observations are taken of the general nature of lubrication provided, i. e., whether or not the grease folds over the bearing, channels, slings away from the bearing, tends to "ball up," etc. Then heat is applied to the bearing as it continues to rotate at the same speed so as to gradually raise the temperature of the bearing

50 until the grease fails to lubricate (the breakdown point) or until a temperature of 300° F. is reached in about 40 minutes from the start of the test. Beginning at a bearing temperature of 100° F., observations of performance are recorded for every 25° F. temperature rise or for any significant development such as texture change, expansion in volume, air entrainment, channelling, leakage, melting and consequent thinning, separation, discoloration, vaporization, etc. After completing the run, the bearing is removed and cooled; and grease remaining on the bearing is examined for texture and consistency change, discoloration, etc. and compared with the original grease. The results obtained are compared with those secured 60 in the same test on a standard premium ball and roller bearing grease of known excellent performance; and the performance of the test grease is rated on a comparative basis as E for excellent, G for good, A for adequate, F for fair and P for poor.

The low temperature torque test of the foregoing table is essentially a measure of the resistance of the grease to congealing and of its ability to afford proper lubrication under extremely low temperature conditions, such as are

encountered in aircraft at very high altitudes. The apparatus employed for the test consists essentially of a vertically mounted hollow spindle with a No. 204K Conrad type 8-ball bearing mounted on the bottom, and a drum on which is wrapped a coiled line for applying torque mounted on the top. The bearing packed with a 60% capacity charge of the grease to be tested is clamped at the inner race to the spindle, while the outer race is clamped immovably to a stationary cup within which the bearing is inserted. The assembly is inserted with the lower bearing end in a low temperature bath containing isopropyl alcohol, and the desired temperature of the bath and bearing is attained by dropping Dry Ice in the bath. The drum and drum extension carried at the upper end of the hollow spindle and protruding from the bath are held in vertical position by a tapered roller bearing. The line coiled around the drum extends over a pulley to a container into which the desired weights are added to apply the torque load to the hollow spindle to thereby cause rotation of the spindle and inner race of the bearing with respect to the fixed outer race. A time of not less than two hours is utilized to cool the bearing to the test temperature, and an additional soaking period at the test temperature is permitted such that the test is not run until three hours from the start of cooling. When the desired bearing temperature and soaking period are attained, a 2000 gram-centimeter torque load is applied in both clockwise and counterclockwise directions, and the number of seconds for one rotation in each direction is observed and the readings averaged.

The torque breakdown machine test is designed to evaluate the lubricating properties of greases used for the lubrication of anti-friction bearings. Two standard 3.9370 inch Timken tapered roller bearings packed with about 25 g. each of the grease under test, and a standard Federal Precision Ball Bearing No. 1211 packed with about 32 g. of the grease are employed, the packed bearings being weighed before test. In the test of each bearing, the bearing is assembled on a motor driven shaft supported by pillow blocks within a bearing housing mounted within an insulated chamber, with a system of levers connected to register any movement of the bearing housing in grams on a platform scale, whereby both the starting torque and the running torque can be measured. The insulated chamber is equipped with a copper coil tubing for the circulation of a cooling or heating medium, and also with an insulated cover equipped with an electric heater and a motor driven fan, whereby the temperature of the chamber and bearing under test can be accurately controlled. The test of the Timken bearings at 80° F. is made at 900 R. P. M., and the test of the Federal bearing at 80° F. is made at 1750 R. P. M., each for a period of two hours. The instant the motor driving the test bearing is started, the first torque reading is recorded as the starting torque. Then running torque and temperature readings of the bearing are recorded at one minute intervals for the first 30 minutes, and at 10 minute intervals for the remaining 1½ hours, while the temperature within the chamber is adjusted to maintain the bearing temperature within 2° of 80° F. At the end of the run, the bearing is removed from the housing and weighed, whereby the weight of the grease remaining on the bearing can be computed. The weight of the grease on the housing

is also determined; and grease leakage (grease escaping from both the bearing and housing) is determined by actual weight measurement or by difference. A visual inspection is made of the grease remaining on the bearing to ascertain whether any structure or texture change has taken place; and the penetration of a sample of the grease taken from the bearing after test is compared with the original penetration of the grease. A second test procedure is conducted on the same machine in this manner, except that in this case the temperature of the chamber and of the bearing is raised gradually from an initial 80° F. to a temperature of 250° F. at the end of an hour. The test is then run at 250° F. for an additional two hours before terminating the test. Similar readings are made as previously described. The results thus obtained are compared with those secured in the same tests on a standard premium ball and roller bearing grease of known excellent performance; and overall lubricating performance of the test grease is generally reported on the basis of this comparison as E for excellent, G for good, F for fair and P for poor.

The foregoing Tables I and II show that the phosphated castor oil soap greases of the present invention show advantageous and, in certain respects, unusual properties. The sodium, lithium and sodium-calcium greases have high dropping points, with the lithium base grease having the unusual dropping point above 500° F. Most of the greases tested by the dynamic shear test show excellent to fair resistance to working down; and practically all of the greases showed excellent performance in the rigorous grease breakdown and torque breakdown machine tests. A sample of the 3:1 sodium-calcium grease containing 0.5% by weight of diphenylamine gave adequate lubrication in a 168 hour continuous run at 228° F. in the torque breakdown machine using a Federal ball bearing. In addition to the tests listed, tests were made on the Timken E. P. Machine on the sodium base grease with various loads ranging from 10 to 45 pounds OK being obtained, which indicates that the phosphated castor oil soap greases possess extreme pressure characteristics.

#### EXAMPLE II

The following example is listed as representative of a lithium base grease of phosphated castor oil possessing excellent low temperature and lubricating properties which adapt it for specialized ball and roller bearing uses. 100 grams of water, 375 grams of an acid-treated light pressed distillate paraffin base lubricating oil having an SUS viscosity at 100° F. of 101, and 370 grams of the above mentioned commercial phosphated castor oil having a phosphorus content of 4.54% by weight, a neutralization number of 146, a saponification number of 301, and an iodine number of 80 were charged to the grease kettle and heating and stirring started. When the temperature of the kettle contents reached 196° F., 470 grams of a 10.1% aqueous lithium hydroxide solution were slowly added over a period of ½ hour and an additional 50 grams of rinse water then introduced. Saponification proceeded for 1 hour at 200–202° F., when the temperature was raised to about 300° F. for dehydration. With the temperature maintained at 301–304° F. over a period of about 2 hours, 1700 grams of di-2-ethylhexyl sebacate having an SUS viscosity at 100° F. of 68 and a pour point below –80° F. were gradually added to bring the grease to de-

sired consistency and to thus obtain about a 4:1 mixture of the synthetic oil with the paraffin base lubricating oil in the final product. The heat was then cut and the product gradually cooled with continued stirring, during which time 13 grams of phenyl alpha-naphthylamine in 50 grams of the paraffin base oil and 0.1 gram of a suitable dye were added. The resulting product was drawn at 225° F. to obtain a hard gel-like orange-colored grease having the following calculated composition:

| Per cent by weight                    |       |
|---------------------------------------|-------|
| Lithium soap of phosphated castor oil | 14.8  |
| Glycerine                             | 1.4   |
| Paraffin base lubricating oil         | 14.8  |
| Di-2-ethylhexyl sebacate              | 68.5  |
| Phenylalphanaphthylamine              | 0.5   |
| Dye                                   | 0.002 |

Typical tests obtained on this grease are set forth in the following Table III.

Table III

|                                                |                       |
|------------------------------------------------|-----------------------|
| Dropping point, °F.                            | Over 500              |
| Penetration, ASTM, 77° F.:                     |                       |
| Unworked                                       | 142                   |
| Worked                                         | 286                   |
| Free alkali (LiOH), per cent                   | 0.05                  |
| Free fatty acid (as oleic), per cent           | 0.13                  |
| Lithium soap, per cent                         | 14.8                  |
| Appearance                                     | Hard, gel-like orange |
| Lubrication—grease breakdown machine—          |                       |
| R. T. to 300° F.                               | A                     |
| Lubrication—torque breakdown machine:          |                       |
| Federal bearing, 80° F.                        | E                     |
| Federal bearing, 80-250° F.                    | E                     |
| Timken bearing, 80° F.                         | E                     |
| Timken bearing, 80-250° F.                     | E                     |
| Low temperature torque—minus 97° F., sec./rev. | 11.1                  |
| Oil separation test—50 hr. at 212° F.:         |                       |
| Separation, per cent                           | 5.2                   |
| Evaporation, per cent                          | 0.18                  |

The oil separation test is described in Army-Navy Aeronautical Specification AN-G-3a, Low Temperature Lubricating Grease, page 5, March 6, 1943. This is a measure of the resistance of the grease to oil bleeding and evaporation. In this test 10 grams of the grease are placed in a weighed 60 mesh screen cone supported from the rim of a weighed 100 milliliter beaker so that the pointed bottom of the screen cone containing the grease is substantially above the bottom of the beaker. This assembly is then placed in a gravity convection oven maintained at 212° F. for a period of 50 hours. At the end of that period, the assembly is removed, cooled in a desiccator, and the beaker and cone weighed together and the beaker weighed separately. The final weight of the beaker minus the initial weight of the beaker divided by the initial weight of the grease sample times 100 is reported as per cent bleeding. The initial weight of the beaker plus cone and grease minus the final weight of the beaker plus cone and grease divided by the initial weight of the grease sample times 100 is reported as per cent evaporation.

The foregoing tests, including the exceptionally high dropping point above 500° F., the satisfactory yield, the excellent low temperature torque (operable at -97° F. and probably at lower temperatures), the low oil separation and evaporation at 212° F. for a light oil as employed, and the excellent lubricating properties for ball and roller bearings over wide ranges of temperature show that this is a premium type of grease of unusual character.

## 10 EXAMPLE III

The following example is listed as typical of a premium type lithium base grease prepared from a mixture of a major proportion of the mentioned commercial phosphated castor oil with a minor proportion of a conventional fatty acid, such as stearic acid, particularly for the production of a grease having exceptional low temperature properties in addition to providing excellent lubrication over a wide temperature range.

324 grams of phosphated castor oil of the character specified above, 110 grams of triple pressed stearic acid, 310 grams of an acid-treated light pressed distillate paraffin base lubricating oil having an SUS viscosity at 100° F. of 101, 200 grams of water, and 513 grams of a 10.1% aqueous lithium hydroxide solution were charged to a grease kettle and heating and stirring started. Saponification was effected at a temperature of 160-190° F. over a period of 2½ hours. Then the temperature was raised rapidly to above 300° F. and maintained at about 311-324° F. for 2 hours to effect dehydration. 930 grams of di-2-ethylhexyl sebacate were then added slowly over a period of 4 hours with continued stirring as the temperature dropped to about 220° F. with 8.6 grams of phenylalphanaphthylamine included in the final portion of the added di-2-ethylhexyl sebacate. During continued stirring and as the temperature dropped to about 180° F., 100 grams of a blend of the di-2-ethylhexyl sebacate with the paraffin base oil in the ratio of 3:1 and containing 0.5 grams of phenylalphanaphthylamine were added, followed by an additional 50 grams of the 3:1 blend containing 0.25 grams of phenylalphanaphthylamine. The grease was drawn at a temperature of 174° F. and a final product of a brown smooth glossy buttery medium feather grease obtained, having the following calculated composition:

| Per cent by weight                    |      |
|---------------------------------------|------|
| Lithium soap of phosphated castor oil | 17.3 |
| Lithium stearate                      | 6.0  |
| Di-2-ethylhexyl sebacate              | 56.0 |
| Paraffin base lubricating oil         | 18.6 |
| Glycerine                             | 1.5  |
| Phenylalphanaphthylamine              | 0.5  |
| Excess LiOH                           | 0.1  |

The following tests were made on this grease in comparison with the Ordnance Department, U. S. Army Specification 2-134, for Low Temperature Instrument Grease, October 8, 1948.

Table IV

|                                                                       | 2-134 Spec. | Grease of Ex. III |
|-----------------------------------------------------------------------|-------------|-------------------|
| Dropping Point, °F.                                                   | 300 min.    | over 500          |
| Penetration ASTM, 77° F.:                                             |             |                   |
| Unworked                                                              |             |                   |
| Worked                                                                | 260-340     | 198               |
| Free Alkali (LiOH), per cent                                          |             | 0.07              |
| Free fatty acid (oleic), per cent                                     |             | 0.30              |
| Oil separation—30 hrs. at 212° F., per cent                           | 5 max.      | 2.09              |
| Moisture Test—10 sec. immersion                                       | (1)         | passes            |
| Oxidation—Norma-Hoffmann Bomb:                                        |             |                   |
| (a) 110 p. s. i., 210° F., 400 hrs., lbs. drop per 100 hrs.           | 5 max.      | 3                 |
| (b) copper catalyzed, 110 p. s. i., 210° F., 20 hours                 | (2)         | passes            |
| Low Temperature torque—67° F., 2000 g. cm., 3 g. of grease, sec./rev. |             | 1.7               |
| Working Stability (100,000 strokes):                                  |             |                   |
| Penetration, ASTM, 77° F. Original (unworked)                         |             | 198               |
| Final                                                                 |             | 267               |
| Dynamic Water Resistance Loss, per cent                               |             | 0.25              |

<sup>1</sup> No clouding or emulsification.

<sup>2</sup> No change in grease or stain on copper.

The moisture test as set forth in the foregoing 2-134 Specification is made by taking ½ to 1

gram of the grease on the end of a stirring rod and immersing for 10 seconds in water in a 200 milliliter beaker. During the period of immersion, the water is observed visually to detect any appearance of cloudiness or other evidence of emulsification of the grease.

The Norma-Hoffmann oxidation test is a measure of the resistance to oxidation of lubricating greases when stored under static conditions for long periods of time, as when coated in thin films on anti-friction bearings, motor parts, etc. In this test, five four-gram samples of the grease are put in flat sample dishes and placed in a stainless steel bomb sealed with a lead gasket in an atmosphere of oxygen under an initial pressure of 110 pounds per square inch at a temperature of 210° F. The pressure drop in pounds within the bomb is then recorded at intervals of 100 hours up to 400 hours or until a pressure drop of 55 pounds per square inch occurs.

The copper catalyzed test of the foregoing table is conducted in the same apparatus, except that a strip of copper is partially immersed in the grease sample. At the end of 20 hours at 210° F. the grease is examined for decomposition or any change in color or consistency, and the copper strip is examined for evidence of corrosion or stain.

The Working Stability test is described in the Army-Navy Aeronautical Specification AN-G-25 for Low Temperature Aircraft Lubricating Grease, October 9, 1947, and is a measure of the texture stability of the grease under shearing stress. In this test a mechanical worker consisting of a cylinder filled with the grease sample to be tested and containing a plunger plate having approximately 270 holes of  $\frac{1}{16}$  inch diameter each is employed, and the plunger is worked back and forth through the grease at the rate of 60 double strokes per minute until 100,000 double strokes have been completed. The final penetration of the worked grease is then taken and compared with the original unworked sample.

The dynamic water resistance test of the foregoing table is that described in Army-Navy Aeronautical Specification AN-G-25, Low Temperature Aircraft Lubricating Grease, Item F-4f, October 9, 1947. This measures the resistance of the grease against being washed out of the bearing in the presence of water. Briefly, the test involves the 204K Conrad ball bearing mentioned above pack with 4 grams of the grease and clamped in a tight fitting housing which allows the inner race to rotate. The latter is mounted on a horizontal shaft and rotated at 600 R. P. M. while a fine stream of distilled water is directed against the end plate of the bearing housing just above the outer opening of the bearing housing. This operation is continued for one hour, when the loss in weight of the dried bearing is then reported as grease loss; and this loss in weight divided by the weight of the grease used in packing the bearing is reported as the percent loss.

The tests of the foregoing table show that this grease easily passes the difficult requirements of the 2-134 Specification. In addition, the high dropping point, the very low time required for one revolution at -67° F. in the low temperature torque test, and the excellent working stability and water resistance of this grease make it outstanding.

Another batch of this lithium base grease of the same formulation was tested in comparison with a conventional lithium base low temperature grease prepared from hydrogenated castor oil

and now on the market, with the results shown in Table V.

Table V

| 5                                                | Conventional<br>Li base Low<br>Temperature<br>Grease | Present<br>Li base<br>Grease |
|--------------------------------------------------|------------------------------------------------------|------------------------------|
| Dropping Pt., °F.....                            | 366.....                                             | 457                          |
| Mean Hertz Load.....                             | 20.....                                              | 37                           |
| Cu corrosion, Norma-Hoffmann Bomb.....           | positive<br>corrosion.                               | no stain.                    |
| Salt spray (100 hrs., 95° F.), percent rust..... | 50 to 60.....                                        | 10:15                        |

The mean Hertz load test is made with the so-called four-ball EP machine as described in the U. S. Naval Engineering Experiment Station Report on Cooperative Evaluation of EP Lubricants, May 3, 1946. This machine comprises essentially a ball pot in which three  $\frac{1}{2}$  inch diameter bearing balls SKF Grade 1, are locked in place by a lock ring and nut. A vertical driving shaft terminating in a ball chuck holder, into which is inserted a ball chuck containing a fourth bearing ball of the same type, extends downwardly into the ball pot so that the fourth ball rotates as it is pressed against the three stationary balls. The ball pot is attached to a mounting disc supported on a thrust bearing, so that the ball pot assembly is free to rotate about its vertical axis; and the ball pot assembly is forced upwardly to engage the balls at predetermined pressures by means of weights applied to a counterweighted lever arm acting through a pressure pin, step bearing and cross-head, the latter supporting the said thrust bearing. In each run, the balls are coated with the grease under test; and the vertical shaft is driven at 1800 R. P. M. for 10 seconds at an applied load. The three balls in the ball pot assembly are then removed for measurement of the scars formed by rubbing of the top or fourth ball on the three lower balls. A new set of four balls is used for each run. This is a measure of the extreme pressure properties of the grease and the empirical figures of the table set forth the so-called extreme pressure value, termed the mean Hertz load, which latter is based on a relationship between the wear-load diagram obtained with the lubricant tested and that of a theoretically perfect lubricant, as described by the so-called Hertz line of elastic deformation. Each determination requires 20 to 27 ten-second runs at prescribed increasing loads up to welding, with subsequent measurement of wear-spot diameters formed on the test balls. The division of a factor, supplied for each applied load, by the wear-spot diameter is made; and the results are averaged to yield a numerical evaluation of the extreme pressure properties of the grease. A higher numerical value represents a closer approach to the theoretically perfect lubricant.

The salt spray test is designed to evaluate the ability of a coating of the grease to protect metal specimens, such as boiler steel specimens, against corrosion in the presence of salt or sea water spray. In this test the metal specimens coated with the protective layer of the grease under test are supported at a 45° angle in an enclosed salt spray box held in an inclined position. An atomizer consisting of two nozzles arranged at right angles is mounted in the lower portion of the inclined box, one nozzle being connected to a source of clean compressed and water-saturated air under a pressure of 12-15 pounds per square inch, with the other nozzle opening into the bottom of the box to draw salt solution up through

this nozzle, atomizing it in the form of a very fine mist. An inclined baffle is mounted between the atomizer and the specimens under test to keep the spray from impinging directly on the specimens. A synthetic sea water solution is used as the salt spray, this synthetic sea water solution being prepared as follows. A stock solution containing 10 grams of KCl, 45 grams of KBr, 550 grams of MgCl<sub>2</sub>·6H<sub>2</sub>O and 110 grams of CaCl<sub>2</sub>·6H<sub>2</sub>O with sufficient distilled water to make 1 liter, is prepared. Twenty milliliters of this stock solution is then mixed with 23 grams of NaCl and 8 grams of Na<sub>2</sub>SO<sub>4</sub>·10H<sub>2</sub>O, and with sufficient distilled water to make up to 1 liter. As shown by the table, the operation is continued for 100 hours at 95° F., and then the specimens are removed and the percentage area of the specimens coated by rust is determined.

As shown by the foregoing Table V, this lithium base grease of the present invention has a higher dropping point, higher load carrying capacity (mean Hertz load), greater resistance to salt spray, and better copper corrosion protection than the premium type of lithium base low temperature grease now employed.

While the foregoing examples illustrate preferred types of greases prepared from the commercial phosphated castor oil, which consists roughly of about equal proportions of phosphated castor oil with unmodified castor oil, it is to be understood that advantageous types of greases as well as improved liquid lubricants can be prepared from phosphated castor oil alone, or phosphated hydrogenated castor oil alone, or mixtures thereof. Likewise, the various other mentioned phosphated soap-forming hydroxy fatty acids or their glycerides can be used in a similar manner. In order to obtain the advantages of the phosphated type of soap in the preparation of lubricants or greases of the present invention, it is desirable to employ as the soap-forming carboxylic acid or glyceride constituents a mixture containing at least about 25% by weight of the phosphated hydroxy fatty acid or glyceride, with the balance being composed of unmodified hydroxy fatty acid or glyceride, or conventional soap-forming fatty acid or glyceride, or mixtures thereof.

Obviously many modifications and variations of the invention as hereinbefore set forth may be made without departing from the spirit and scope thereof, and therefore only such limitations should be imposed as are indicated in the appended claims.

We claim:

1. A lubricating grease comprising an oleaginous liquid lubricating base containing in excess of 5% and up to 45% by weight based on the grease of a metal soap of a phosphated soap-forming material selected from the group consisting of a phosphated soap-forming hydroxy fatty acid and a phosphated soap-forming hydroxy fatty acid glyceride sufficient to thicken said lubricating base to a gel-like consistency.

2. A lubricating grease comprising an oleaginous liquid lubricating base thickened to a gel-like consistency with a proportion in excess of 5% and up to 45% by weight based on the grease of a metal soap of phosphated castor oil having the formula



where M is an alkali metal.

3. A lubricating grease according to claim 2, wherein the oleaginous liquid lubricating base consists of a major proportion of an oil-soluble high molecular weight high boiling liquid aliphatic dicarboxylic acid ester within the lubricating oil viscosity range and possessing lubricating properties and a minor proportion of a mineral lubricating oil, and M of the metal soap is lithium.
4. A lubricating grease according to claim 3, wherein the said aliphatic dicarboxylic acid ester is di-2-ethylhexyl sebacate.
5. A lubricating grease comprising an oleaginous liquid lubricating base thickened to a gel-like consistency with a proportion in excess of 5% and up to 45% by weight based on the grease of lithium soap consisting of a major proportion of the lithium soap of phosphated castor oil and a minor proportion of lithium soap of a saturated soap-forming fatty acid.
6. A lubricating grease according to claim 5, wherein the lithium soap of the saturated soap-forming fatty acid is lithium stearate.
7. A lubricating grease comprising an oleaginous liquid lubricating base thickened to a gel-like consistency with a proportion in excess of 5% and up to 45% by weight based on the grease of a sodium soap of phosphated castor oil.
8. A lubricating grease comprising an oleaginous liquid lubricating base thickened to a gel-like consistency with a proportion in excess of 5% and up to 45% by weight based on the grease of a mixed base sodium-calcium soap of phosphated castor oil.
9. A lubricating grease comprising an oleaginous liquid lubricating base containing in excess of 5% and up to 45% by weight based on the grease of a metal soap of a phosphated hydrogenated castor oil sufficient to thicken said lubricating base to a gel-like consistency.
10. A lubricating grease comprising an oleaginous liquid lubricating base as the major constituent and a proportion in excess of 5% and up to 45% by weight based on the grease of metal soaps of a mixture consisting essentially of phosphated castor oil and castor oil to thicken said lubricating base to a gel-like consistency, said phosphated castor oil constituting at least 25% by weight of said mixture.
11. A lubricating grease according to claim 10, wherein said mixture consists essentially of about 45-50% by weight of phosphated castor oil and 55-50% by weight of castor oil, and the metal of said soaps is lithium.
- 55 EDWIN C. KNOWLES.  
ONEY P. PURYEAR.  
GEORGE W. ECKERT.
- 60 REFERENCES CITED
- 60 The following references are of record in the file of this patent:
- UNITED STATES PATENTS
- | Number    | Name              | Date           |
|-----------|-------------------|----------------|
| 2,128,946 | Katzman           | Sept. 6, 1938  |
| 2,142,998 | Chittick          | Jan. 10, 1939  |
| 2,228,658 | Farrington et al. | Jan. 14, 1941  |
| 2,294,817 | Van Dijck         | Sept. 1, 1942  |
| 2,345,734 | Dickey et al.     | Apr. 4, 1944   |
| 2,356,754 | Farrington et al. | Aug. 29, 1944  |
| 2,450,222 | Ashburn et al.    | Sept. 28, 1948 |
| 2,450,254 | Puryear et al.    | Sept. 28, 1948 |
| 2,450,255 | Puryear et al.    | Sept. 28, 1948 |
- 70 FOREIGN PATENTS
- 75 Number Country Date
- 424,380 Great Britain Feb. 20, 1935